

June 29, 1943.

**W. H. FURNESS**  
**MANUFACTURE OF CUPRAMMONIUM RAYON**

2,322,801

Filed May 1, 1940



INVENTOR:  
William Henry Furness  
BY Syme, Woodward & Lechner  
ATTORNEYS.

## UNITED STATES PATENT OFFICE

2,322,801

## MANUFACTURE OF CUPRAMMONIUM RAYON

William H. Furness, Haddonfield, N. J., assignor  
to American Rayon Company, Inc., Riverton,  
N. J., a corporation of New Jersey

Application May 1, 1940, Serial No. 332,696

2 Claims. (Cl. 18—54)

This invention relates to the art of manufacturing cuprammonium rayon and other cellulose products from cuprammonium cellulosic solutions, and its nature, objects and advantages will be best understood from the following.

Generally speaking, in the spinning of cuprammonium rayon, for example, the cellulosic spinning solution is prepared and spun through suitable spinnerets into a caustic soda setting bath, and the bundle of filaments, after leaving the setting bath and while in a plastic state, is subjected to a sulphuric acid wash for the purpose of removing caustic soda, copper and ammonia from the filaments. It is later subjected to water washing to remove acid and soluble salts, and then to a drying operation.

This general procedure has several drawbacks. One of these is the difficulty and expense of recovery of chemicals. For example, the caustic soda, during the process, is converted into sodium sulphate, and the solutions are so dilute and the expense of recovering the sodium sulphate is so great that the solution is discarded. The case is the same with the ammonia, which is converted into ammonium sulphate during the process. With respect to the copper, the usual practice has been to recover it by the addition of caustic soda to form basic copper sulphate, and here again sodium sulphate is formed and the solution of sodium sulphate is so dilute that it is discarded, with the resultant loss in caustic soda consumed to form the sodium sulphate. Another difficulty is that relatively large quantities of sulphuric acid are required.

The primary object of the present invention is to overcome these difficulties and to make it possible to recover for re-use, the caustic soda, copper and ammonia, in a very simple and effective manner.

In carrying out my invention I prefer to employ the cellulosic spinning solution from wood pulp, according to my copending application Serial No. 129,820, filed March 9, 1937 (now Patent No. 2,225,431, dated December 17, 1940). Briefly, the wood pulp is first subjected to caustic soda solution to effect certain changes therein, after which surplus caustic soda solution is expressed and the treated wood pulp, together with ammonia and tetrammonio copper sulphate are used to prepare the spinning solution. For this spinning solution, the caustic soda employed should be in the ratio of 2 mols for each mol of copper sulphate, and the ammonia should be in the ratio of from about 7

to about 8 mols, although the quantity employed may be greater.

This solution is spun into a caustic soda setting bath which is relatively dilute, containing from about 25 to 45 grams per liter NaOH, depending upon such factors as the concentration of cellulose in the spinning solution.

According to my invention, the freshly spun filaments, after leaving the setting bath and prior to the sulphuric acid wash, are treated to remove practically all of the ammonia, the bulk of the caustic soda, and a substantial portion of the copper, for reasons which will hereafter appear. In order to accomplish this, I operate on a continuous basis, as diagrammatically illustrated in the accompanying drawing wherein the reference character A denotes a source of cellulosic spinning solution, which is pumped through spinnerets B into the caustic soda setting bath C, from which the bundle of filaments, through the use of suitable guides, not shown, is led to a revolving cage D, which operates to continuously advance the bundle of filaments in the form of a helix. In the order named, the helix is subjected to a hot water wash, then to the sulphuric acid wash, then to a water wash, and finally to a drying operation carried out, if desired, on the cage. For convenience in separation of the treatment or wash liquids and for other reasons, the bundle of filaments, after leaving the hot water wash section, is led from the cage over a roller E and then back to the cage, from which point it is advanced in the form of a helix as before.

35 The hot water wash has the effect of removing the bulk of the caustic soda, practically all of the ammonia and a substantial part of the copper from the filaments. Although the water need not be hot, I prefer hot water for the reason that caustic soda is more soluble in hot water than in cold and further, it is desirable to use no more water than will accomplish the desired end, and the results can be obtained with a smaller volume of water, if hot. The water dilutes the ammonia in and on the filaments, thus tending to cause cupric hydroxide (resulting from the action of the caustic soda of the setting bath) to come out of solution, and the continual application of the water physically removes ammonia and copper hydroxide. Moreover, the heat drives off some of the ammonia as gas, thus further decreasing the concentration of ammonia and increasing the tendency of the copper to come out of solution. The copper hydroxide is given an opportunity to settle out

of the collected wash liquor, is separated and washed to remove any caustic soda present, in which condition it is fit for re-use as herein-after pointed out. By virtue of the evaporation of ammonia and the washing away of ammonia by the water, for all practical purposes all of the ammonia is removed from the filaments, which is important for reasons hereinafter appearing.

The advantages of removing the bulk of the caustic soda before the filaments are subjected to the sulphuric acid wash, are as follows. In the first place, since caustic soda is used in the setting bath, it is highly desirable from the standpoint of effectiveness, to recover the caustic soda, as such, so that it can be returned to the spinning bath. This can not be effectively done if the caustic soda is removed in the acid section, because as a result of the reactions occurring in that section, the caustic soda is consumed in forming sodium sulphate, and the cost of recovering it is so expensive as to be prohibitive. I can readily make the caustic soda in the hot water wash liquor available for re-use in the system by boiling it to drive off the ammonia therein and, if needed, to drive off sufficient water to increase the concentration of caustic soda to the point where the concentrated liquor can be returned to the setting bath storage tank. In the next place, much less acid is required by my process because the amount of caustic soda remaining in the filaments to be removed by the acid is relatively very small. Furthermore, the amount of sodium sulphate formed in my process is such that it constitutes no difficulty in the system and if it objectionably builds up, it can be, if desired, removed as set forth in my copending application, Serial No. 332,694, filed May 1, 1940.

The advantages of removing a substantial part of the copper from the filaments in the hot water wash section are as follows. Less acid is required, for there is less copper to remove. Moreover, an excess of sulphuric acid over the theoretical requirements is always needed in the acid wash section for obvious reasons, and consequently the acid wash liquor always contains some free acid, in addition to the sodium sulphate and the copper sulphate produced as a result of the reactions occurring in the acid wash section. Now, I propose to recover the copper sulphate in the acid wash liquor by adding cupric hydroxide which converts the soluble copper sulphate into the insoluble basic copper sulphate which can be separated as by sedimentation, centrifuging, filtering or the like. By removing copper from the filaments in the hot water wash section, in the form of cupric hydroxide, I have thus available cupric hydroxide for use in neutralizing the excess sulphuric acid in the acid wash liquor, the reaction between the sulphuric acid and the cupric hydroxide being to form some copper sulphate, which, in addition to the copper sulphate already present in the wash liquor, is recovered, as above set forth, by the addition of the acid wash liquors of further amounts of cupric hydroxide sufficient to convert all of the copper sulphate into basic copper sulphate. I prefer to remove at least sufficient copper as cupric hydroxide in the hot water wash section to neutralize the excess or free sulphuric acid in the acid wash liquor. If more cupric hydroxide is removed in the hot water wash section, it is available for use in the acid wash liquor to convert copper sulphate into basic copper sulphate.

The advantages of removing practically all of

the ammonia from the filaments in the hot water wash section are as follows. As before, this lessens the amount of acid required. In the next place, the presence of substantial ammonia in the filaments reaching the acid wash section would result in the formation in that section of ammonium sulphate which would be present in the acid wash liquor. This would interfere with the removal of copper sulphate from the acid wash liquor in the form of basic copper sulphate, by the use of cupric hydroxide. By the hot water wash the ammonia in the filaments, if not entirely removed, is reduced to such a small amount as not to interfere with the removal of the copper sulphate as basic copper sulphate. Furthermore, ammonia is needed to convert the basic copper sulphate into tetrammonio copper sulphate, and the ammonia removed by the hot water washing operation is very easily recoverable as ammonia water and is used as a source of ammonia for the conversion of basic copper sulphate into tetrammonio copper sulphate. The products of the reaction between basic copper sulphate and ammonia are tetrammonio copper sulphate and cupric hydroxide, the latter being separated in any of the ways described. The tetrammonio copper sulphate is used in the manufacture of the cellulosic spinning solution, and the copper hydroxide obtained by the reaction between basic copper sulphate and ammonia, is available for removing copper sulphate from the acid wash liquor.

Another advantage of removing ammonia from the filaments and recovering the same from the wash liquors for re-use as indicated is that thereby the final supernatant liquors are freed of ammonia. These final supernatant liquors are ultimately re-used in the system by returning them to the spinning bath system. This is of advantage because ammonia in the setting bath interferes with good spinning. In this connection I employ a relatively dilute caustic soda setting bath which is more effective for spinning, the less the ammonia present therein.

There are traces of chemicals in the water wash section following the acid wash, but the amount is so small as to be negligible.

Instead of using a single cage, two cages may be used, the first cage constituting the hot water wash section, and the second cage the acid section, followed by water washing and drying. It is also obvious that the principles of the invention can be carried out with other apparatus.

The water in the hot water wash section should be hot enough to effectively remove the bulk of the caustic soda and preferably not so hot as to convert the copper hydroxide to the black cupric oxide. To use water that hot would be uneconomical, since the copper hydroxide can be used as such.

It is of course obvious that the length of the hot water section should be such that ample opportunity is provided for the filaments to be subjected to the hot water wash sufficiently long to accomplish the desired removal of caustic soda, ammonia and copper. The period will vary with the variation in denier of the filaments. Likewise the acid wash section should be long enough to serve the functions for which the acid is employed.

The complete system by which I manufacture cuprammonium rayon and recover chemicals, etc., is described and claimed in my copending application Serial No. 332,694, filed May 1, 1940. That system advantageously employs the present invention but since the present invention is capable

of independent use, I herein claim it apart from the general system.

What I claim is:

1. In a continuous system of spinning and treating cellulosic products such as rayon, staple, films and the like, from cuprammonium cellulosic solutions, in which the filaments, films or the like, are spun into a caustic soda setting bath and afterwards subjected to a sulphuric acid wash, the process which comprises subjecting the freshly spun material intermediate the setting bath and the acid wash and while in a plastic state to a hot water wash to remove substantially all of the caustic soda and the ammonia, and a substantial portion of the copper as cupric hydroxide, separating the cupric hydroxide and washing it, and using the washed cupric hydroxide to remove acid in the used wash liquors.

2. In a continuous system of spinning and treating cellulosic products such as rayon, staple, films and the like, from cuprammonium cellulosic solutions, in which the filaments, films, or the like are spun into a caustic soda setting bath and afterwards subjected to a sulphuric acid wash and to a final water wash, the process which comprises subjecting the freshly spun material intermediate the setting bath and the acid wash and while in a plastic state to a hot water wash to remove substantially all of the caustic soda and the ammonia, and a substantial portion of the copper as cupric hydroxide, separating the cupric hydroxide and washing it, and using the washed cupric hydroxide to remove free acid and copper sulphate in the used wash liquors, thereby producing basic copper sulphate for use in making fresh spinning solutions.

WILLIAM H. FURNESS.